# EUROPEAN PATENT APPLICATION

(11) **EP 0 572 670 A1**
(43) Date of publication of application: **08.12.1993**
(21) Application number: 92919639.2
(22) Date of filing: 10.09.1992
(51) Int. Cl.: D01F 6/62

(54) **POLYCAPROLACTONE STAPLE FIBER AND PRODUCTION**

(30) Priority: 13.09.1991 JP 263237/91
(71) Applicant: UNITIKA LTD., Amagasaki-shi Hyogo 660 (JP); NIPPON UNICAR COMPANY LIMITED, Chiyoda-ku Tokyo 100 (JP)
(72) Inventor: MOCHIZUKI, Masatsugu, Central Research Inst., Kyoto 611 (JP); KANMURI, Yoshihirom, Central Research Inst., Kyoto 611 (JP); TAKAHASHI, Syuji, Central Research Inst. of, Kyoto 611 (JP); KANEMOTO, Naoki, Central Research Inst. of, Kyoto 611 (JP); INOUE, Takashi, 222-1-203, Imainishimachi, Kanagawa 211 (JP)
(74) Representative: Le Vrang, Klaus
(86) International application number: JP9201161
(87) International publication number: WO9306267

(57) **Abstract**

A polycaprolactone staple fiber having a tensile strength of 3.0 g/denier or above, the number of crimps of 8-35/25 mm and a crimp ratio of 5.0 % or above. A biodegradable polycaprolactone staple fiber having excellent crimp characteristics and strength can be provided by melt spinning a polycaprolactone with a melt flow rate of 25 g/10 min or less at 200 to 300 °C, cooling the formed fiber, applying thereto a spinning finish, taking up, if desirable, the treated fiber, stretching the same in one or more steps at room temperature to 60 °C, mechanically crimping the stretched fiber, applying thereto a short fiber finish, drying the treated fiber, and cutting the dried fiber.

## Description

### TECHNICAL FIELD

The present invention relates to staple fibers made of polycaprolacton and a method of producing same.

### BACKGROUND ART

Hitherto, synthetic fibers, such as polyolefin, polyamide, aromatic polyester, and vinylon, have been used as material fibers for domestic sundry supplies including sanitary items, such as diapers and sanitary napkins, disposable hand towels, wiping cloths, and the like, mainly from economical standpoints. However, these fibers have no self-digesting property and this poses a problem that such articles, if left outdoor after use, will lead to various environmental pollutions. As such, with those disposable items, there has been no alternative but burning them after use.

One solution to such a problem may be to use a self-digesting (microbially degradable or biodegradable) material.

Self-digesting polymers have been well known including polysaccharides, such as cellulose and chitin, proteins, such as catgut and regenerated collagen, polypeptides (polyamino acids), microbial polyesters produced by microorganisms in nature, such as poly-3 -hydroxybutyrate or a copolymer thereof, and synthetic aliphatic polyesters, such as polyglycolide, polylactide and polycaprolacton.

In particular, cotton, a natural cellulose, and rayon, a regenerated cellulose, are known to be comparatively inexpensive materials of the biodegradable type. However, these materials have the disadvantage that although they are subject to biodegradation, the rate of their biodegradation is comparatively low. For example, when rayon is buried in a landfill of refuse wherein it has little chance of being sufficiently mixed with or contacted with soil, the progress of degradation of the rayon is further retarded, which presents a serious problem. Another deficiency is that such cellulose material is hydrophilic, which fact makes the material unsuitable for use in applications in which hydrophobic nature is required of the material, such as for example cover stock (surface sheeting) for sanitary napkins for which a short-fiber nonwoven fabric of polyolefin is currently used. Further, with such material, which is non-thermoplastic, heat sealing cannot be effected and, therefore, the material is not available as a thermal bonding fiber.

Attempts to produce fibers from other polymers present several problems. Production of fibers from some polymers requires wet spinning. Use of some other polymers involves very high material costs which result in a high cost of manufacture. In some other cases, fibers obtained have no sufficient strength.

Among others, polycaprolacton is a synthetic polymer which is comparatively inexpensive but yet completely biodegradable, and which can be melt spun into a fiber. However, no report has ever been made that short fibers having any specific strength and crimp characteristics were actually produced. Assumably, the melting point of polycaprolacton which is as low as about 60 °C may be a factor which has made it difficult to produce fine fibers from polycaprolacton and to impart given crimp characteristics to fibers, if any, produced from polycaprolacton. Another reason may be that it has been difficult to commercially obtain a high-molecular weight polycapro lacton having good spinning processing characteristics.

In an attempt to provide an inexpensive self-digesting material there has been proposed a polyethylene-starch blend. Already, a film formed from a Straight-chain low-density polyethylene blended with about 6 % starch has been put to practical use in a limited area of application, such as shopping bags.

However, short fibers produced from such a Starch-blended polyethylene are of poor performance characteristics, with unsatisfactory mechanical properties, such as strength and crimp characteristics, and, therefore, can hardly be used in general sundry and/or domestic applications. Further, polyethylene is not biodegradable, even though starch is biodegradable. This fact tells that a starch blended polyethylene does not provide any fundamental solution.

### DISCLOSURE OF THE INVENTION

It is an object of this invention to provide a polycaprolacton-based staple fiber which is comparatively inexpensive, has excellent crimp characteristics and high strength sufficient for practical use, and is microbially degradable, and a method of producing same.

The subject matter of the invention is as follows:
( 1 ) A polycaprolacton-based staple fiber having a tensile strength of not less than 3.0 g / denier, the number of crimps of 8 to 35 / 25 mm, and a crimp percentage of not less than 5.0 %.
( 2 ) A method of producing a polycaprolacton-based staple fiber which comprises melt spinning a polycaprolacton having a melt flow rate (g / 10 min) of not more than 25 as measured according to J I S K 6760, at temperatures of 200 to 300°C, air-cooling the resulting filament, then applying spinning lubricant to the filament, drawing the filament, via a winding stage once or immediately without winding, in a temperature range of from room temperature to 60°C in one stage or more than one stage, subsequently mechanically imparting crimps to the drawn filament, applying a short fiber lubricant, followed by drying, and then cutting.

It is to be noted that the staple fiber of the invention includes a mixture staple fiber containing a small quantity of other aliphatic polyester and/or polyolefin within such limits as can meet the foregoing characteristic requirements.

The invention will now be described in further detail.

The polycaprolacton used in the invention has a melt flow rate (g / 10 min) of not more than 25, preferably not more than 10, as measured according to J I S K 6760. If the melt flow rate exceeds 25, it is impracticable to provide a staple fiber having the strength and crimp characteristics intended to be achieved by the invention.

The staple fiber of the invention can be produced by melt spinning a polycaprolacton having a high degree of polymerization, subjecting the resulting filament to drawing and mechanical crimping, and then cutting.

The temperature for melt spinning may vary according to the melt flow rate of the polycaprolacton but it must be not less than 200°C but not more than 300°C. If the spinning temperature is less than 200 °C, it is difficult to carry out melt extrusion. If the temperature exceeds 300°C, decomposition will become pronounced so that it is difficult to obtain a staple fiber having high strength and good crimp characteristics.

The spinning velocity may be greater as the filament denierage is finer. The upper limit of the spinning velocity may vary according to cooling conditions, etc., but it may be on the order of 2000 m / min for 1 denier, 1600 m / min for 3 denier, and 300 m / min for 20 denier.

The melt spun multifilament is air-cooled and is then given spinning lubricant. The spinning lubricant is to impart cohesive force and antistatic property to filament strands, and for this purpose a conventional spinning lubricant may be used.

Filament strands having spinning lubricant applied thereto are drawn in one stage or more than one stage in a temperature range of from room temperature to 60°C after they are wound up once or without being wound up. The draw ratio applicable varies according to the required performance characteristics of the staple fiber to be produced, but usually it is set so as to provide a fiber elongation at breakage of not more than 100 %, preferably 30 to 90 %.

Nextly, filament strands drawn as described above are given a crimpage of 8 to 35 crimps / 25 mm, preferably 10 to 30 crimps / 25 mm, according to the stuffing box method, forced heated gear method, or high-speed air jet stuffing method, and are then cut to a length of 20 to 100 mm. In this case, if the number of crimps is less than 8 / 25 mm, unopened fiber spots are likely to occur in the carding stage. If the number is greater than 35 / 25 mm, neps are likely to develop. Also, it is necessary to arrange that crimp percentage is not less than 5.0 %. If the crimp percentage is less than 5.0 %, when staple fibers are subjected to carding in the next stage, density irregularities are likely to occur with the card web due to insufficient cohesiveness.

For the purpose of imparting crimps by the forced heated gear method, yarn strands, prior to their entry into the crimper, should be preheated to 40-60 °C in a warm water bath or otherwise and, only after that, they should be passed through the crimper under a nip pressure of 1.0 to 3.5 kg/cm² and a force-in pressure of 1.0 to 3.5 kg/cm² (it is possible to increase the number of crimps and crimp percentage by increasing fill density).

Filament strands subjected to crimping are then passed through the stage for application of short fiber lubricant for preventing static charging during carding operation, and a drying stage, and finally they are cut by a cutter into staple fibers.

For the short fiber lubricant, any lubricant similar to spinning lubricant may be used, but a lubricant which provides no large cohesive power is employed so as to enhance satisfactory opening behavior during carding operation.

The staple fiber of the invention, obtained in this way, has excellent crimp and strength characteristics, and favorable microbial degradability, as stated earlier.

The single yarn fineness of staple fiber is usually 1 to 20 denier.

The staple fiber of the invention is spun into yarns according to conventional spinning process and then processed into knitted or woven fabrics, or processed into short fiber nonwoven fabrics via dry or wet process.

In this way, according to the invention, a microbially degradable staple fiber is provided which has good crimp and strength characteristics suitable for practical uses and which is of hydrophobic nature and has thermal bondability.

Knitted and woven fabrics and/or nowoven fabrics using the staple fiber of the invention are suitable for use in sanitary applications, such as cover stock (surface sheet) for disposable diapers, sanitary napkins, disposable hand towels, and pads. They are also suitable for use as such domestic sundry items as wiping cloths and base fabrics for happing materials. Such items made of the staple fiber of the invention, after use, may be left as such in any environment in which microorganisms are present (in earth or underwater), and can be completely biodegraded in a given period of time, it being thus possible to compost those wastes.

### Description of Example

The following example is given to further describe the present invention.

In the example, tensile strength and elongation characteristics were measured according to J I S L 1015. Specimens were buried in the earth and were removed after two months for examination. Where the staple fiber had lost its primary configuration, the fiber was judged as having good biodegradability.

A polycaprolacton having a melt flow rate of 4 was melt spun through a spinneret having 30 spinning holes of 0.3 mm dia. each at a spinning temperature of 260°C and spinning speed of 1200 m/min.

Air at room temperature was blown to the melt spun filament for cooling. Then, to the filament was applied an aqueous emulsion lubricant composed principally of mineral oil and aliphatic ester and containing an antistatic agent and an emulsifying agent in blend therewith. The undrawn filament was wound up once.

Nextly, the undrawn filament was drawn in two stages at room temperature so that total draw ratio would be 2.4 ( = 1.1 × 2.18 ). Then, the drawn filament was preheated in a warm water bath at 50 °C, whereafter it was introduced into a push-in gear type crimper (nip pressure: 3.0 kg / cm², push-in pressure: 3.0 kg / cm²) in which it was subjected to crimping. Subsequently, the filament was lubricated with a lubricant similar to spinning lubricant and subjected to drying, being then cut to a length of about 51 mm. Thus, a staple fiber having a single yarn fineness of 3 denier was obtained.

The obtained staple fiber had a tensile strength of 4.2 g / denier, an elongation at break of 72.1 %, the number of crimps of 25.8 / 25 mm, and a crimpage of 8.2%. The staple fiber was well fitted for passage through carding process, and it also exhibited satisfactory microbial degradability.

## Claims

1. A polycaprolacton-based staple fiber having a tensile strength of not less than 3.0 g / denier, number of crimps of 8 to 35 / 25 mm, and a crimp percentage of not less than 5.0 %.

2. A staple fiber as claimed in claim 1, wherein the number of crimps of the staple fiber is 10 to 30 / 25 mm.

3. A staple fiber as claimed in claim 1, wherein the length of the staple fiber is 20 to 100 mm.

4. A staple fiber as claimed in claim 1, wherein the single yarn fineness of the staple fiber is 1 to 20 denier.

5. A method for producing a polycaprolacton-based staple fiber which comprises melt spinning a polycaprolacton having a melt flow rate (g / 10 min) of not more than 25 as measured according to J I S K 6760, at temperatures of 200 to 300°C, air-cooling the resulting filament, then applying spinning lubricant to the filament, drawing the filament, via a winding stage once or immediately without winding, in a temperature range of from room temperature to 60°C in one stage or more than one stage, subsequently mechanically imparting crimps to the drawn filament, applying a short fiber lubricant, followed by drying, and then cutting.

6. A method as claimed in claim 5, wherein spinning is carried out in a spinning speed range of 300 to 2000 m/ min and wherein drawing is carried out in a draw ratio such that the elongation at break of the fiber is not more than 100 %.

7. A method as claimed in claim 5, wherein crimping is carried out according to the push-in heated gear method and wherein filaments strands are preheated before their entry into a crimper and are then passed through the crimper under conditions of nip pressure of 1.0 to 3.5 kg / cm² and push-in pressure of 1.0 to 3,5 kg / cm².
